

June 24, 1969

B. ANCELLE ET AL  
BLEACHING PULP HAVING HIGH CONSISTENCY WITH  
OZONE HAVING MOISTURE CONTENT NEAR 100 %  
Filed April 28, 1966

3,451,888



FIG. 1



FIG. 2



FIG. 3

INVENTOR.  
*Bernard Ancelle*  
BY *Marcel Plancon*  
BY *Tourouer and Browly*  
*Attorneys*

1

3,451,888

BLEACHING PULP HAVING HIGH CONSISTENCY  
WITH OZONE HAVING MOISTURE CONTENT  
NEAR 100%

Bernard Ancelle and Marcel Plançon, Lyon, France, as  
signors to Progil, Paris, France, a corporation of France  
Filed Apr. 28, 1966, Ser. No. 545,919  
Claims priority, application France, Apr. 30, 1965,  
45,940

Int. Cl. D21c 9/10, 9/16

U.S. Cl. 162—65

8 Claims

**ABSTRACT OF THE DISCLOSURE**

A method of bleaching paper-making pulp which is 15  
an aqueous slurry having a dry consistency of 30–65%  
by passing a gaseous stream containing ozone which has  
a moisture content near 100% through the pulp.

The present invention relates to a method of bleaching  
paper pulp utilizing ozone. More particularly, it re-  
lates to the use of wetted ozonized air as a bleaching  
agent.

In classical processes, bleaching is effected on cellulosic  
pulps, in a combined way, with active products such  
as chlorine, chlorine dioxide, soda and sodium hypo-  
chlorite. But applied techniques are long and expensive  
as they need several treatment stages and extensive  
equipment.

It has been tried to bleach paper pulps by means of  
dry ozonized air. This method reduced corrosion prob-  
lems and makes the working process easier. Moreover,  
since ozone is produced only by the action of an elec-  
tric discharge upon air, the bleaching agent is continually  
available without any raw material stocking. But it has  
been noted that such a treatment gives rise to a very  
important pulp drying. This disadvantage is the more  
serious as, when starting from a dry gaseous flow, the  
humidity rate of the whole system varies progressively  
to the reaction between cellulosic material and ozonized  
air. So drying is more or less pronounced in the different  
parts of the pulp and it results in irregular non-homo-  
geneous bleaching. It is not possible to stop this phenom-  
enon by lengthening treatment time, since this results in  
a whiteness reversion. Moreover, the pulp becomes  
strongly degraded, especially at the points where drying  
is the most pronounced, and it shows characteristics  
incompatible with market requirements.

The present invention has for an object the provision  
of a bleaching process, very easy to carry out, and leading  
to an improved whiteness, keeping at the same time  
pulp quality.

Also, the invention provides for a given whiteness  
equal to the one of a classical bleaching, the improvement  
of pulp characteristics.

The applicants have found the above results are ob-  
tained by the action of an ozonized air flow saturated with  
moisture upon the pulp to be bleached. Indeed it has  
been established that, when the process is carried out  
with a wetted gaseous flow, the moisture rate of the  
system remains constant and optimal, contrary to what  
happens with dry ozonized air. There is neither local  
drying nor cellulose degradation and bleaching is homo-  
geneous and regular.

In its most general form, the process according to the  
invention comprises passing a gaseous flow, coming from  
an ozonizer and titrating 2.5 to 18 mg. O<sub>3</sub>/liter, prefer-  
ably 4 to 16 mg./liter, into a saturator/moistener, then  
sending it as it escapes from the apparatus at a rate of  
50 to 500 liter/hour, preferably 100 to 300 liter/hour

2

during a time of ½–2½ hours, preferably 1 to 2 hours,  
to a shredded paper pulp, with a dryness of 30–65%,  
having a pH near neutrality and maintained at a tem-  
perature of 20 to 30°C.

The moisture state of the gaseous flow is an essential  
element of the process according to the present invention.  
The ozonized air must have a relative moisture  
near 100%. In any case it is necessary that the moisture  
content be the highest possible in order to avoid any  
drying variation of the pulp in treatment and to give to  
bleaching its efficiency maximum.

The ozonized gaseous flow according to the invention  
may be constituted not only by air, as this is considered  
during this description, but also by oxygen.

Azone titre and gaseous rate may be selected in the  
present invention field with regard to the variables in-  
herent to the used installation without being prejudicial  
to the obtained result: indeed experiment has shown that  
the important factor in this field is the weight of used  
20 ozone per time unit. For example a fairly similar white-  
ness will be obtained in carrying out the process during  
the same time: A gaseous flow at a rate of 300 l./hr.,  
titrating 6.10 mg. O<sub>3</sub>/l. (that is 1830 mg. O<sub>3</sub>/hr.); a  
gaseous flow at a rate of 200 l./hr., titrating 9.30 mg.  
25 O<sub>3</sub>/l. (that is 1860 mg. O<sub>3</sub>/hr.).

Treatment time may vary in the limits of 30 minutes  
to 2 hours 30 minutes according to the conditions se-  
lected in the field in order to give a maximum treatment  
efficiency. This may easily be established with regard to  
30 the selected gaseous rate and/or ozone titre, so as to  
obtain the desired bleaching degree. For example, a white-  
ness, "Elrepho" of 60 may be obtained:

in 1 hr. with a gaseous rate of 300 l./hr. titrating 6.10  
35 mg. O<sub>3</sub>/l.;  
in 1½ hr. with a gaseous rate of 100 l./hr. titrating  
6.50 mg. O<sub>3</sub>/l.

In the same way a whiteness "Elrepho" of 71 may be  
40 obtained:

in 1½ hr. with a gaseous rate of 200 l./hr. titrating  
9.4 mg. O<sub>3</sub>/l.;  
in 2 hr. with a gaseous rate of 200 l./hr. titrating 7  
45 mg. O<sub>3</sub>/l.;  
in 2½ hr. with a gaseous rate of 200 l./hr. titrating  
4 mg. O<sub>3</sub>/l.

The charts of FIGS. 1, 2 and 3 allow one to determine  
in an easy way gaseous flow rate, ozone titre and treat-  
50 ment time which may be chosen with regard to the de-  
sired result.

On these charts are plotted, as abscissa, the time in  
hours of ozonized air treatment, and, as ordinate, the  
whiteness of the obtained pulp, measured in index  
55 Elrepho. Each one of the charts has 3 curves *a*, *b* and *c*  
plotted for ozonized air rates and ozone titres given in  
the following table:

|    |                            | Fig. 1 | Fig. 2 | Fig. 3 |
|----|----------------------------|--------|--------|--------|
| 60 | Ozonized air rate (l./hr.) | 100    | 200    | 300    |
|    | Ozone titre (in mg./l.):   |        |        |        |
|    | <i>a</i> -----             | 6.5    | 4.0    | 2.9    |
|    | <i>b</i> -----             | 11.7   | 7.0    | 4.5    |
|    | <i>c</i> -----             | 15.5   | 9.4    | 6.1    |

65 The bleaching method according to the present in-  
vention is limited neither by raw material nature nor by  
the process used for paper pulp fabrication. For ex-  
ample, pulps obtained from wood of resinous or long  
70 leaf trees and prepared by soda, sulfite or sulfate proc-  
ess fit quite well to the method according to the in-  
vention.

Pulp dryness degree is an important factor for the use of the method according to the present invention. Tests have shown the optimal value varies with regard to pulp nature, cooking and refining degrees. Our experiments have established the most favourable dryness rate is generally between 30 and 65%. For example, a beech kraft pulp, treated during 2 hours, at 20° C. with an ozonized air flow saturated with moisture, at a rate of 100 l./hr. and titrating 15.5 mg. ozone/liter has the following Elrepho whiteness values according to pulp concentration:

|                        |    |    |      |    |
|------------------------|----|----|------|----|
| Dryness, percent.....  | 27 | 51 | 62   | 78 |
| Elrepho whiteness..... | 68 | 80 | 79.5 | 58 |

A eucalyptus kraft pulp, treated at a rate of 200 l./hr. with an ozone concentration of 9.5 mg./l. has the following values:

|                        |    |    |    |    |
|------------------------|----|----|----|----|
| Dryness, percent.....  | 30 | 40 | 50 | 60 |
| Elrepho whiteness..... | 66 | 75 | 70 | 59 |

The pulp must preferably have a pH the nearest possible to neutrality, but a pH varying between 6 and 7.5 is not prejudicial to process application according to the present invention.

The most favourable reaction temperature is from 20 to 30° C. A comparative study has shown bleaching decreases when temperature increases. For example, a beech kraft pulp with 60% of dryness treated with an ozonized air stream of 100 l./hr., saturated with moisture and titrating 15.5 mg. O<sub>3</sub>/l. gives the following Elrepho whiteness values, according to reaction temperature:

| Treatment time | Elrepho whiteness |       |        |
|----------------|-------------------|-------|--------|
|                | 30 min.           | 1 hr. | 2 hrs. |
| Temperature:   |                   |       |        |
| 25° C.....     | 58                | 78    | 87     |
| 45° C.....     | 50                | 71    | 85     |
| 65° C.....     | 36                | 50    | 71     |

The ozonized air stream saturated with moisture should be at the same temperature as that at which the pulp is maintained during reaction. Moreover, it must be taken care that the cellulosic material does not undergo notable temperature increase during ozonization. For this reason the equipment may possibly be provided with a cooling system.

Practically, the process according to the present invention offers a great ease in application since it consists of sending ozonized air to paper pulp in an only working stage. The treatment may be made in a discontinuous way, but also in a continuous one, which is interesting for industrial applications. Indeed experiment shows the method according to the invention may be made in a continuous way without residual ozone in the air at the bleaching tower outlet.

Though the process according to the invention may advantageously replace classical bleaching methods, it may alternatively be used in association with these classical methods. Thus, ozone treatment may be inserted into a bleaching sequence in several stages, ozonization being able to come before or to follow the usual treatments with hydrogen peroxide, hypochlorite or chlorine and soda.

The following examples, given in a non-limitative way, show how the process according to the invention may be applied.

#### EXAMPLE 1

A sample A of 25 g. of pine kraft unbleached pulp having a dryness rate of 40% (10 g. of dry extract) is shredded and put into a glass flask provided with an inlet tube and a gas recovery tube. The pulp has a pH of 7 and is maintained at a temperature of 20° C. An ozonized air stream titrating 15.5 mg./l. ozone is saturated with

moisture at 20° C. in a moistener and enters the flask at a rate of 100 l./hr. The treatment is carried on for 2 hours.

A second identical sample, B, is treated in the same conditions but the ozonized air stream titrates 7.0 mg./l. ozone and is sent to the flask at a rate of 200 l./hr.

The main characteristics of the pulps obtained in this way are summarized in the following table:

|                                  | Non-treated sample | Sample A | Sample B |
|----------------------------------|--------------------|----------|----------|
| (1) Elrepho whiteness.....       | 22                 | 77       | 74       |
| Weight, g./m. <sup>2</sup> ..... | 72.6               | 67.8     | 68.9     |
| (2) Hand*.....                   | 2.18               | 1.88     | 1.93     |
| (3) Tensile length (m.).....     | 3,250              | 4,050    | 4,200    |
| (4) Bursting index.....          | 17                 | 18       | 20       |

(1) AFNOR norm NF Q. 03. 008.  
 (2) AFNOR norm NF Q. 03. 016.  
 (3) AFNOR norm NF Q. 03. 004.  
 (4) AFNOR norm NF Q. 03. 014.

\*The ratio thickness/weight in g./m.<sup>2</sup>.

20 The values obtained for whiteness indexes are the more remarkable as starting paper pulp was especially difficult to bleach since it had a permanganate index of 39.

#### EXAMPLE 2

This example illustrates the very clear superiority of the bleaching with moistened ozonized air according to the present invention, with regard to the known process with dry ozonized air.

30 Two sample series of 50 g. of beech kraft unbleached pulp, of dryness 60% and a pH equal to 7, are treated according to the same working processes as in the Example 1, with an ozonized air flow titrating 15 mg./l. at a rate of 100 l./hr. at 25° C. For the first series the

35 ozonized air is dry; for the second ones the ozonized air is saturated with moisture. The results are given in the following table:

| Treatment time                   | Dry ozonized air |        | Moistened ozonized air |        |
|----------------------------------|------------------|--------|------------------------|--------|
|                                  | 1 hr.            | 2 hrs. | 1 hr.                  | 2 hrs. |
| Elrepho whiteness.....           | 67               | 75     | 73                     | 83     |
| Shopper degree.....              | 14               | 15     | 14                     | 14     |
| Weight, g./m. <sup>2</sup> ..... | 69.4             | 68.3   | 68.3                   | 67.8   |
| Hand*.....                       | 2.05             | 2.05   | 2.14                   | 2.05   |
| Tensile length (m.).....         | 2,550            | 2,450  | 2,700                  | 2,750  |
| Bursting index.....              | 8                | 7.5    | 11                     | 10.5   |
| (5) Tear index.....              | 51               | 41     | 48                     | 42     |

(5) AFNOR norm NF Q. 03. 011.

\*The ratio thickness/weight in g./m.<sup>2</sup>.

50 The above tests make quite clear the two aspects of the greater treatment efficiency with wet ozonized air with regard to bleaching with dry ozonized air:

on the one hand, for the same treatment time, whiteness is fairly improved (respectively 6 and 8 points for 1 and 2 hours of reaction);

55 on the other hand, for the same whiteness, obtained with wet ozonized air, after a treatment time much shorter than in the case of dry ozonized air, pulp characteristics are improved, especially with regard to breakdown length, bursting index and tear index.

It will be obvious to those skilled in the art that various changes may be made without departing from the spirit of the invention and therefore the invention is not limited to what is shown in the drawing and described in the specification.

65 What is claimed is:

1. In a method of bleaching a paper-making pulp by passing a gaseous stream containing ozone through the pulp, the improvement which consists in saturating the 70 gaseous stream with moisture before passing it through the pulp, said pulp being an aqueous slurry having a dry consistency of 30 to 65%.

2. A method in accordance with claim 1 comprising: passing a gaseous mixture of ozone containing 2.5-18 mg. O<sub>3</sub>/liter and having a moisture content near 100%,

to said pulp slurry having a pH of 6-7.5; maintaining the flow of said gaseous mixture for  $\frac{1}{2}$ - $2\frac{1}{2}$  hours; and terminating said flow of gas.

3. A method in accordance with claim 1, wherein said ozone is first generated in an atmosphere which is not saturated with water, and is then provided with said moisture content near 100%.

4. A method in accordance with claim 1, wherein said ozone content is 4-16 mg.  $O_3$ /liter, said flow rate is 50-500 liters/hr., said treatment is carried out for 1-2 hours, said gaseous mixture has a moisture content of 100%, and aid pulp has a pH close to 7, and a temperature of 20-30° C.

5. A method in accordance with claim 1, wherein said gaseous mixture consists essentially of air, water and ozone.

6. A method in accordance with claim 1, wherein

said gaseous mixture consists essentially of oxygen, water and ozone.

7. A method in accordance with claim 1, wherein the temperature of said gaseous mixture is maintained at approximately the same value as that of said pulp.

8. A method in accordance with claim 1 wherein the temperature of said pulp is about 20 to 30° C.

#### References Cited

##### UNITED STATES PATENTS

2,466,633 4/1949 Braebender ----- 162-65

HOWARD R. CAINE, *Primary Examiner.*

U.S. Cl. X.R.

8-111